

## UNITED STATES PATENT OFFICE

DONALD B. BRADNER, OF PHILADELPHIA, PENNSYLVANIA

## ALUMINUM OPHORITE

No Drawing.

Application filed February 21, 1925. Serial No. 10,982.

(GRANTED UNDER THE PROVISIONS OF THE ACT OF MARCH 3, 1883, 22 STAT. L. 625)

The invention described herein may be used by the Government, or any of its officers or employees, in prosecution of work for the Government, or by any other person in the United States, without payment of royalty thereon.

This invention relates to a new explosive composition and more specifically to aluminum ophorite.

10 The term ophorite is applied to a mechanical mixture of metallic magnesium and a perchlorate, which on ignition burns rapidly, yielding intense heat and a sufficient amount of gas for development of high pressures when the material is confined. This material is used in connection with military explosives for the fragmentation of shells and the ignition of a material, such as thermite.

20 Among the objects of this invention is the production of an ophorite mixture which possesses greater effectiveness, power and stability and which can be produced from materials of greater availability than the ophorite previously made.

25 A further object of this invention is the production of an ophorite wherein metallic aluminum is substituted for the magnesium metal of the prior compositions of this character.

30 Aluminum ophorite possesses the following advantages over magnesium ophorite:

35 1. Aluminum metal is more available and can be produced more cheaply than metallic magnesium.

40 2. In magnesium ophorite, the magnesium is employed as coarse cuttings and this affords greater possibility of segregation of the magnesium with consequent failure of the mixture.

45 If finely-divided magnesium be used to counteract this tendency toward segregation, the resulting mixture becomes too sensitive to handle and the rate of explosion is too rapid to ignite the theremite. The aluminum in the ophorite is employed in a finely-divided condition.

50 3. Aluminum ophorite is more stable in storage than magnesium ophorite. There is less tendency for surface oxidation in the former than in the latter.

4. Aluminum ophorite gives more heat per weight of metal, and consequently a smaller charge is required for a given result.

In carrying out my invention I incorporate finely-divided metallic aluminum with a finely-divided oxidizing agent, such as a perchlorate. I prefer potassium perchlorate for this purpose, although other perchlorates, such as that of sodium or ammonium may be substituted, in whole or in part, for the potassium perchlorate.

I find that the source and quality of the aluminum metal is an important factor in the final properties of the mixture. I have found that "flake" aluminum (aluminum foil ground in oil) is most satisfactory for my purpose. Also, the fineness of the perchlorate as well as its freedom from impurities and moisture content are important factors in the effectiveness of the product.

A specific example of preparing my composition is as follows: The aluminum metal, which should be preferably substantially pure and ground so that about at least 80% shall be of 100-200 mesh and containing not in excess of 2% of oil is added to the potassium perchlorate, preferably in a pure and dry condition and of a fineness of at least 150 mesh. The components are used approximately in proportions which will give complete oxidation of the aluminum metal, the theoretical proportions by weight, in which the aluminum and perchlorate are used, being 34.2% aluminum and 65.8% potassium perchlorate, in which the oil is present with the aluminum not in excess of 2%, which react according to the following equation:



The components are mixed separately, and are then placed in a tumble barrel or glass bottle wherein they may be shaken and entirely mixed without heat or friction.

The present invention is not limited to the specific details set forth in the foregoing examples which should be construed as illustrative and not by way of limitation, and in view of the numerous modifications which may be effected therein without departing from the spirit and scope of this invention,

it is desired that only such limitations be imposed as are indicated in the appended claims.

I claim as my invention:

1. An explosive material comprising a mixture of finely ground metallic aluminum foil ground in oil, said oil constituting not in excess of two per cent of the mixture and a perchlorate of an alkali metal.
2. An explosive material comprising a mixture of metallic aluminum foil finely ground in a mineral oil and potassium perchlorate, said oil constituting not in excess of 2% of the mixture.
3. A process for preparing an explosive material comprising mixing finely ground metallic aluminum foil ground in a mineral oil said oil not constituting in excess of two per cent of the mixture and a perchlorate of an alkali metal in proportion for complete oxidization of the aluminum to aluminum oxid by the perchlorate.
4. A process for preparing an explosive material comprising mixing finely ground metallic aluminum foil ground in a mineral oil said oil not constituting in excess of two per cent of the mixture and potassium perchlorate in proportions for complete oxidization of the aluminum to aluminum oxid by the potassium perchlorate.
5. An explosive material comprising a mixture of finely divided metallic aluminum ground in oil, said oil constituting not in excess of two per cent of the mixture and potassium-perchlorate, said aluminum being ground so that at least 80% shall be of 100-200 mesh and the potassium-perchlorate of a fineness of at least 150 mesh.
6. A process for preparing an explosive material comprising mixing finely ground metallic aluminum foil, ground in a mineral oil, and finely ground potassium-perchlorate in proportions of approximately 34.2% of aluminum and 65.8% of potassium-perchlorate, said mixture not containing in excess of 2% of oil.
7. An explosive material comprising a mixture of flake aluminum and a perchlorate of an alkali metal.
8. An explosive material comprising a mixture of flake aluminum and potassium-perchlorate.

DONALD B. BRADNER.